

## UNITED STATES PATENT OFFICE

2,035,740

## TREATMENT OF TEXTILE MATERIALS

Camille Dreyfus, New York, N. Y., and William Whitehead, Cumberland, Md., assignors to Celanese Corporation of America, a corporation of Delaware

No Drawing. Application December 1, 1931,  
Serial No. 578,414

7 Claims. (Cl. 28—1)

This invention relates to the treatment of textile materials, and relates more particularly to the treatment of yarns or fabrics containing organic derivatives of cellulose in order to improve 5 their properties.

An object of our invention is to treat textile materials containing organic derivatives of cellulose with a substance comprising a free higher fatty acid whereby their properties are improved. 10 Other objects of our invention will appear from the following detailed description.

Many substances such as vegetable or mineral oils have been employed for lubricating yarns in order to render them more suitable for winding, 15 fabric forming or other textile operations. However, such oils tend to gum or polymerize with time, so that yarns lubricated with them, when aged, do not run as smoothly as is often desired, in knitting machines and the like. Moreover, acetone soluble cellulose acetate yarn that 20 has olive oil applied thereto and which has been aged for several months, does not deluster evenly when treated with hot aqueous fluids with the result that fabrics formed from such yarn, when 25 dyed or otherwise finished, do not have an even deluster, but obtain streaks that have a luster different from the remaining portions of the fabric.

We have found that oleic acid or other free 30 higher fatty acids form an excellent finish for yarns, filaments, fabrics or other textile materials comprising organic derivatives of cellulose, which has many advantages over finishes previously employed, as will appear below.

35 In accordance with our invention we treat textile materials containing organic derivatives of cellulose after their formation with a substance comprising a free higher fatty acid.

This invention is applicable to the treatment 40 of fine filaments, or a plurality of such fine filaments associated together in the form of yarn or larger filaments such as artificial bristles, horse-hair, straw and the like, and also to fabrics or other articles formed therefrom.

45 Filaments or yarns containing or made of cellulose acetate or other organic derivatives of cellulose such as organic esters of cellulose and cellulose ethers may be treated in accordance with our invention. Examples of other organic esters 50 of cellulose are cellulose formate, cellulose propionate, cellulose butyrate, while examples of cellulose ethers are ethyl cellulose, methyl cellulose and benzyl cellulose.

As stated, in accordance with our invention we 55 treat textile materials with a substance com-

prising a free higher fatty acid. While we prefer to employ oleic acid, other free higher fatty acids containing at least 8 carbon parts of the molecule such as the free fatty acids derived from coconut oil, stearic acid, palmitic acid, ricinoleic acid, or mixtures of two or more of these may be employed. However, we prefer to employ a higher fatty acid which is a liquid or a mixture of such acids, which mixture is in liquid form.

The finish, besides containing the oleic acid or 10 other free higher fatty acids, may contain other ingredients such as diethylene glycol, ethylene glycol, ethyl oxybutyrate, olive oil, coconut oil, mineral oil or a mixture of two or more of these.

The oleic acid or other higher fatty acid may 15 be applied as such, or it may be applied whilst dissolved in an organic liquid, or it may be applied while emulsified in an aqueous liquid containing soaps, Turkey red oil, or other suitable dispersing agents. Examples of volatile solvents 20 for oleic acid are benzene, toluene, xylene, ethyl benzene, trimethyl benzene and gasoline; while examples of relatively non-volatile solvents for oleic acid are monoethyl ether of diethylene glycol, the propyl or butyl ethers of diethylene 25 glycol, mineral lubricating oils and the liquid glycerides of fatty acids.

The finish containing oleic acid or other free 30 higher fatty acid may be applied to the yarns or filaments at the spinning cabinet at which they are formed while in transit to a winding and/or twisting device. However, it may be applied to the yarn during any other textile operation, such as while traveling from package to package or while in the form of hanks. Fabrics 35 may be impregnated with such finish or such finish may be padded thereon in any suitable manner.

The application of the substance containing 40 oleic acid or other free higher fatty acid of textile materials serves many useful purposes, some of which are here given.

The substance containing oleic acid or other 45 free higher fatty acid may be applied to the filaments of organic derivatives of cellulose at the spinning cabinet where they are formed prior to winding and/or twisting, whereby the filaments are lubricated and the yarns formed therefrom are lubricated and therefore are more amenable to winding, knitting or other textile operations. 50 Moreover, the oleic acid prevents or reduces the tendency of the yarns or filaments to develop charges of static electricity. Furthermore fabrics formed from aged yarn that has been treated with oleic acid do not develop uneven luster 55

during dyeing, delustering or other finishing operations.

Another application of this invention is the use of oleic acid or other free higher fatty acid as a constituent of size, which is to be applied to warps of yarns of organic derivatives of cellulose in order to render them capable of withstanding the drastic conditions prevailing during weaving. Fabrics formed from such warps do not develop an appreciable amount of warp streaks after dyeing, delustering and other finishing operations.

A still further application of this invention involves the use of oleic acid and/or other free higher fatty acids to aid the delustering of yarns of organic derivatives of cellulose or fabrics containing the same. Yarns which have been treated with the oleic acid or fabrics containing such treated yarn may be treated with hot aqueous fluids such as aqueous solutions of soap near the boiling point or wet steam, whereupon they readily deluster to form an even subdued luster free of streaks. If a woven fabric made of yarn which has been sized with ordinary size not containing oleic acid or other free higher fatty acid is to be delustered, preferably such size is first removed prior to the application of the oleic acid and the like.

Another important aspect of our invention is in the treatment of old yarn or fabric which has olive oil thereon. Such yarn or fabric when dyed or treated with hot aqueous liquid assumes an uneven deluster. To prevent this, we treat such aged yarn or fabric with a substance containing oleic acid or other suitable free higher fatty acid and then subject the same to hot aqueous baths and thus obtain an even, subdued luster on the fabric or yarn.

In order further to illustrate our invention, but without being limited thereto, the following specific examples are given.

#### Example I

Yarn consisting of filaments of an acetone soluble cellulose acetate of approximately 54.5% combined acetic acid and of 150 denier, 40 filaments and 2.5 turns per inch twist is furnished during a winding operation with rollers, wicks, discs, or other furnishing means with 5% of its weight of the following mixture:

#### Part

|                   |   |
|-------------------|---|
| Castor oil        | 1 |
| Diethylene glycol | 1 |
| Oleic acid        | 1 |

The yarn so finished is found to have improved pliability, greatly enhancing the even appearance of knitted goods therefrom. Such yarns or goods therefrom, irrespective of age and/or conditions of storing, show no progressive change in delustering and dyeing properties and, further, the finish thereon shows practically no polymerization as evidenced by gumming as compared with castor oil or its mixtures with diethylene glycol or other solvent to which free fatty acids such as oleic acid have not been added, similarly applied and exposed.

#### Example II

A yarn similar to that in Example I is furnished by similar means with a 50% solution of oleic acid in the monobutyl ether of diethylene glycol to which has been added 1% of the phospholipide, lecithin. Yarns so finished have the improved knitting qualities, also the uniform dyeing and delustering properties irrespective of age or

conditions of exposure, exhibited by yarns prepared according to the procedure of Example I, and further, have even greater resistance to oxidative and polymerization changes in the finish thereon, which changes would produce gumming which is antagonistic to winding, knitting and like operations and are liable to cause dyeing and delustering changes when dyeing and delustering treatments are subsequently effected.

#### Example III

A fabric comprising yarn of acetone soluble cellulose acetate of approximately 54.5% combined acetic acid, which yarn has been finished with olive oil, peanut oil, tea seed oil, cotton seed oil, or other oils comprising unsaturated fatty acid radicals, during the spinning operations or winding operations conducted thereafter and which yarn is of several different ages, say from 2 to 12 weeks taking the age of the yarn back to the time when finished with the olive or similar oil, is padded to remove size with an emulsion of oleic acid 33%, NaOH 5% and added water 62% at 70° C. After so treating, it is preferable though not always essential to allow the fabric to stand a sufficient time to permit thorough soaking and penetration of the emulsion, the time for such standing will vary according to the nature of the fabric, the closeness of weave and the amount of twist in the yarn therein and so on, but usually soaking times of not more than 4 hours after padding are sufficient. The fabric is then scoured and dyed normally and/or delustered. The fabric thus finished is found to be uniformly dyed and/or delustered, but if not so treated is found to show differences in dyeing and delustering which may be connected with the age of the yarn.

#### Example IV

The following is an example of a size made in accordance with our invention for application to a warp consisting of cellulose acetate yarn.

|              | Percent |
|--------------|---------|
| Gelatin      | 3.2 45  |
| Dextrin      | 6.7     |
| Glycerin     | 0.7     |
| Oleic acid   | 0.7     |
| Benzoic acid | 0.2     |
| Water        | 88.5 50 |

The size is applied to the warp by means of a slasher in an amount equal to 8 to 10% of the weight of the yarn. The warp may then be inserted in a loom and then woven into a fabric.

It is to be understood that the foregoing specific examples are given merely by way of illustration and that many variations may be made therein without departing from the spirit of this invention.

Having described our invention, what we desire to claim and secure by Letters Patent is:

1. Delustered yarns comprising an organic derivative of cellulose finished with an unsaturated fatty acid derivative and aged and which have had applied thereto, at a time no later than the delustering operation, a finish comprising a free higher fatty acid.

2. Delustered yarns comprising cellulose acetate finished with an unsaturated fatty acid derivative and aged which have had applied thereto, at a time no later than the delustered operation, a finish comprising oleic acid.

3. Process of reducing the luster of textile materials containing organic derivative of cellulose yarns previously finished with an unsaturated

- fatty acid derivative and then aged, which comprises treating said materials with a hot delustering fluid in the presence of a free higher fatty acid.
5. 4. Process of reducing the luster of textile materials containing cellulose acetate yarns previously finished with an unsaturated fatty acid derivative and then aged, which comprises treating said materials with a hot delustered fluid in 10 the presence of oleic acid.
5. Process of effecting uniform reduction of luster of textile materials containing organic derivative of cellulose yarns previously finished with an unsaturated fatty acid derivative and 15 then aged, which comprises impregnating the materials with a free higher fatty acid and thereafter subjecting the materials to the action of a hot aqueous delustering liquid.
6. Process of effecting uniform reduction of luster of textile materials containing cellulose acetate yarns previously finished with an unsaturated fatty acid derivative and then aged, which comprises impregnating the materials with a free higher fatty acid and thereafter subjecting the materials to the action of a hot aqueous delustering liquid.
7. Process of effecting uniform reduction of luster of textile materials containing cellulose acetate yarns previously finished with olive oil and then aged, which comprises impregnating the materials with oleic acid and thereafter subjecting the materials to the action of a hot aqueous delustering liquid.

15

15

CAMILLE DREYFUS.  
WILLIAM WHITEHEAD.

## CERTIFICATE OF CORRECTION.

Patent No. 2,035,740.

March 31, 1936.

CAMILLE DREYFUS, ET AL.

It is hereby certified that error appears in the printed specification of the above numbered patent requiring correction as follows: Page 2, second column, line 71, claim 2, and page 3, first column, line 9, claim 4, for "delustered" read delustering; and that the said Letters Patent should be read with these corrections therein that the same may conform to the record of the case in the Patent Office.

Signed and sealed this 28th day of April, A. D. 1936.

Leslie Frazer

(Seal)

Acting Commissioner of Patents.

- fatty acid derivative and then aged, which comprises treating said materials with a hot delustering fluid in the presence of a free higher fatty acid.
5. 4. Process of reducing the luster of textile materials containing cellulose acetate yarns previously finished with an unsaturated fatty acid derivative and then aged, which comprises treating said materials with a hot delustered fluid in 10 the presence of oleic acid.
5. Process of effecting uniform reduction of luster of textile materials containing organic derivative of cellulose yarns previously finished with an unsaturated fatty acid derivative and 15 then aged, which comprises impregnating the materials with a free higher fatty acid and thereafter subjecting the materials to the action of a hot aqueous delustering liquid.
6. Process of effecting uniform reduction of luster of textile materials containing cellulose acetate yarns previously finished with an unsaturated fatty acid derivative and then aged, which comprises impregnating the materials with a free higher fatty acid and thereafter subjecting the materials to the action of a hot aqueous delustering liquid.
7. Process of effecting uniform reduction of luster of textile materials containing cellulose acetate yarns previously finished with olive oil and then aged, which comprises impregnating the materials with oleic acid and thereafter subjecting the materials to the action of a hot aqueous delustering liquid.

15

15

CAMILLE DREYFUS.  
WILLIAM WHITEHEAD.

## CERTIFICATE OF CORRECTION.

Patent No. 2,035,740.

March 31, 1936.

CAMILLE DREYFUS, ET AL.

It is hereby certified that error appears in the printed specification of the above numbered patent requiring correction as follows: Page 2, second column, line 71, claim 2, and page 3, first column, line 9, claim 4, for "delustered" read delustering; and that the said Letters Patent should be read with these corrections therein that the same may conform to the record of the case in the Patent Office.

Signed and sealed this 28th day of April, A. D. 1936.

Leslie Frazer

(Seal)

Acting Commissioner of Patents.

CERTIFICATE OF CORRECTION.

Patent No. 2,035,740.

March 31, 1936.

CAMILLE DREYFUS, ET AL.

It is hereby certified that error appears in the printed specification of the above numbered patent requiring correction as follows: Page 2, second column, line 71, claim 2, and page 3, first column, line 9, claim 4, for "delustered" read delustering; and that the said Letters Patent should be read with these corrections therein that the same may conform to the record of the case in the Patent Office.

Signed and sealed this 28th day of April, A. D. 1936.

Leslie Frazer

(Seal)

Acting Commissioner of Patents.